

## UNITED STATES PATENT OFFICE

2,157,322

## MAGNESIUM ALLOY

Fritz Christen, Zurich-Altstetten, Switzerland

No Drawing. Application March 5, 1938, Serial  
No. 194,221. In Switzerland December 30,  
1937

1 Claim. (Cl. 75—142)

The invention relates to a pre-alloy (masterbatch alloy) for producing and improving magnesium alloys which latter customarily contain 5.9-10% aluminium, 0.2-5% zinc, 0.2-2% manganese and often 0.1-1.2% silicon as well.

The magnesium alloys hitherto known do not exhibit a sufficient resistance to corrosion and have not a sufficient hardness, particularly if such alloys are employed for producing elements 10 which are subjected to varying working temperatures.

A further disadvantage resides in that although by altering the additives it is certainly possible to obtain an increasing tensile strength, 15 the malleability is reduced.

The object of the present invention is to eliminate these disadvantages of such alloys. With this object in view and in accordance with the purpose to which the alloys are put, the pre-alloy 20 according to the invention is added in an amount lying within the range of 4-12% whereby the hardness and the mechanical strength of the resultant alloy is increased and the possibility of further working for example by forging, rolling 25 and the like is favorably influenced.

The pre-alloy according to the invention has the following composition:

|                          | Percent   |
|--------------------------|-----------|
| (1) Aluminium            | 33 - 40   |
| (2) Zinc                 | 23.5-16.5 |
| (3) Copper               | 17.5-14.5 |
| (4) Manganese            | 3 - 6     |
| (5) Nickel               | 1 - 3     |
| (6) Cobalt               | 6 - 4     |
| (7) Chromium             | 0.5 - 0.9 |
| (8) Molybdenum           | 0.5 - 0.9 |
| (9) Magnesium (constant) | 15        |

In accordance with the use of rising or falling 40 percentages of the corresponding elements 1 and 2, 3 and 4, 5 and 6, 7 and 8 and in accordance

with the choice of the percentage of the pre-alloy which is added to the alloy, the properties of the latter are effected in respect of strength, behaviour under the action of heat, sliding and frictional properties, and capacity for being 5 worked.

## Example

The pre-alloy consisting of the above composition and produced in a suitable manner is 10 added in a preheated condition at about 100° C. to the actual magnesium melt or to the melt of the magnesium alloy if an alloy is to be improved, the percentage added being within the prescribed limits. The added pre-alloy slowly dissolves in 15 the melt.

During this melting operation the customary flux rises to the surface and covers the melt. When everything has become fluid the melt is thoroughly stirred and heated further to 20 800-900° C.

Then the crucible is removed from the furnace and after waiting some minutes for it to cool down to the casting temperature of 700-750° C., the alloy is cast into pigs or moulded blocks. 25

## I claim:

As an article of new manufacture for use in the production of magnesium alloys, a pre-alloy of the following composition:

|                          | Percent   |
|--------------------------|-----------|
| (1) Aluminium            | 33 - 40   |
| (2) Zinc                 | 23.5-16.5 |
| (3) Copper               | 17.5-14.5 |
| (4) Manganese            | 3 - 6     |
| (5) Nickel               | 1 - 3     |
| (6) Cobalt               | 6 - 4     |
| (7) Chromium             | 0.5 - 0.9 |
| (8) Molybdenum           | 0.5 - 0.9 |
| (9) Magnesium (constant) | 15        |

FRITZ CHRISTEN. 40